

# UNITED STATES PATENT OFFICE.

ALBERT D. CONLEY AND ELTING C. STILLWELL, OF BALTIMORE, MARYLAND,  
ASSIGNORS TO JAMES P. HOOPER, OF BALTIMORE, MARYLAND.

## PROCESS OF TREATING REGENERATED CELLULOSE ARTICLES.

1,371,300.

Specification of Letters Patent.

Patented Mar. 15, 1921.

No Drawing.

Application filed June 3, 1919. Serial No. 301,568.

To all whom it may concern:

Be it known that we, ALBERT D. CONLEY and ELTING C. STILLWELL, citizens of the United States, residing at Baltimore city, 5 in the State of Maryland, have invented certain new and useful Improvements in Processes of Treating Regenerated Cellulose Articles, of which the following is a specification.

- 10 The present invention pertains to the improvement of structures, such as films, threads or filaments, or fabrics prepared from viscose and consisting of, or comprising, regenerated cellulose, for the purpose of 15 removing the hard feel and imparting a soft silky feel, and added flexibility and suppleness, and for the improvement of the luster thereof, so as to more closely simulate natural silk.
- 20 The films or filaments, according to the present invention, may be prepared in any desired way, by subjecting the viscose solution to the action of a suitable setting bath, and the invention has been found to produce especially favorable results, by treating 25 filaments produced by squirting viscose solution into a hot substantially saturated solution of ammonium sulfate, although threads prepared from viscose by the employment of other setting baths may be similarly treated for the improvement thereof.

The threads produced by squirting viscose solution into hot ammonium sulfate solution 35 may be then cleaned in a hot substantially saturated solution of sodium bisulfite. The articles are then washed in water, and are then subjected, according to the present invention, to the action of soluble castor oil 40 and a caustic alkali. The regenerated cellulose structures may be first subjected to a bath containing 10%, more or less, of soluble castor oil, which bath may be followed by a bath containing 5%, more or less, of caustic 45 soda, this again being followed by a 10% solution of the soluble castor oil. Ammonium hydroxid or alkaline earth hydroxid, such as calcium hydroxid or barium hydroxid, and in some instances, borates, or perborates, 50 oxids or peroxids of the alkali or alkaline earth metals, may be used in the place of some or all of the caustic soda. These substances may replace about a chemically equivalent quantity of caustic soda. In case 55 peroxids are used, nascent oxygen is liber-

ated, which in addition to bleaching, acts to destroy objectionable sulfur compounds remaining. For most purposes, sodium hydroxid or ammonium hydroxid is preferred.

As a modified procedure, a single solution 60 containing the soluble oil and the alkali hydroxid may be mixed, and the threads, etc., treated therewith. The process may also be employed in conjunction with various other processes which have been devised for the 65 treatment of artificial silk.

In the operation of the process, the alkali hydroxid or the alkaline earth metal hydroxid react with the soluble castor oil to produce a soap. The formation of the soap 70 in the pores of, or in the interior of, or while in contact with the threads, as produced by the alternate subjection to the action of the soluble castor oil bath and the alkaline hydroxid bath (alkali hydroxid or alkaline 75 earth metal hydroxid) has produced rather better results than the use of a mixed bath.

The above description refers particularly to the employment of soluble castor oil. Attention is called, however, to the fact that 80 other soluble oils, particularly soluble fatty oils, may be employed with the production of satisfactory results. Sulfonated cotton-seed oil, sulfonated linseed oil, etc., are mentioned as examples.

The invention, as herein described, embraces the product or products produced in accordance with the process herein described, as well as the process itself.

The caustic alkali seems to unite with the 90 oil to produce a soap to some extent, although we do not wish to confine the invention to this as being the only action which takes place. The successive treatment seems to give better results than when the alkali 95 and oil are first mixed together, for some reason.

Having described our invention, we claim,

1. A process which comprises setting viscose in a hot solution containing ammonium sulfate, subjecting it to a cleaning bath, and then while still wet to the action of alternate baths containing soluble castor oil and sodium hydroxid. 100
2. A process of treating regenerated cellulose structures by subjecting them to alternate baths containing soluble castor oil and sodium hydroxid. 105
3. A process which comprises alternately 110

subjecting regenerated cellulose articles to the action of a bath of solution of soluble fatty oil and a bath of an alkaline hydroxid solution.

5 4. A process which comprises subjecting regenerated cellulose articles to the action of a soluble fatty oil and an alkaline hydroxid.

5 5. A process which comprises subjecting 10 regenerated cellulose articles to the action of a soluble fatty oil and an alkali hydroxid.

6. A process which comprises subjecting cellulose articles made from viscose, to the 15 action of a solution comprising an alkaline hydroxid and a soluble oil.

7. A process which comprises subjecting regenerated cellulose to the action of a soluble oil and to the action of a solution capable of forming a soap with the soluble oil 20 and containing nascent oxygen.

8. A process which comprises subjecting regenerated cellulose to the action of a soluble oil in water and to the action of a solution of a caustic alkali containing nascent 25 oxygen.

9. A process which comprises subjecting regenerated cellulose to the action of a soluble oil in water and to the action of a solution containing nascent oxygen.

30 10. A process which comprises subjecting

regenerated cellulose to the action of a soluble oil in water and to the action of a solution capable of forming a soap with the soluble oil.

11. A process of improving regenerated 35 cellulose articles by forming in them a soap caused by the action of an alkali hydroxid upon a soluble oil which has been previously absorbed by the structure.

12. A product comprising regenerated cel- 40 lulose articles impregnated with the reaction products of a soluble oil and an alkaline hydroxid.

13. A regenerated cellulose structure containing the reaction products of an alkali 45 hydroxid and a soluble fatty oil which have reacted while in contact with the said structure.

14. A regenerated cellulose structure containing the reaction products of a caustic 50 alkali and soluble castor oil.

15. A process which comprises subjecting regenerated cellulose articles to the action of a solution of soluble castor oil, and to the 55 action of a solution of a caustic alkali.

In testimony whereof we affix our signatures.

ALBERT D. CONLEY.  
ELTING C. STILLWELL.